

1,352,696.

A. ROBERTS.

ART OF COOKING COAL.

APPLICATION FILED DEC. 1, 1919.

Patented Sept. 14, 1920.



# UNITED STATES PATENT OFFICE.

ARTHUR ROBERTS, OF EVANSTON, ILLINOIS, ASSIGNOR TO AMERICAN COKE AND CHEMICAL COMPANY, OF CHICAGO, ILLINOIS, A CORPORATION OF MAINE.

## ART OF COKING COAL.

1,352,696.

Specification of Letters Patent. Patented Sept. 14, 1920.

Application filed December 1, 1919. Serial No. 341,696.

*To all whom it may concern:*

Be it known that I, ARTHUR ROBERTS, a citizen of the United States, residing at Evanston, county of Cook, and State of Illinois, have invented certain new and useful Improvements in the Art of Coking Coal, of which the following is a specification.

This invention has to do with certain improvements in the art of coking coal for the production of coke, and the recovery of by-products. The present invention concerns itself particularly with a process for the production of coke and by-products from certain classes of coals.

The present invention has particular reference to improvements in this art whereby it is possible to produce satisfactory metallurgical coke from a large class of coals which have heretofore been classed as "non-coking". By way of introduction, I may state that for many years it has been well understood that metallurgical coke could be produced by the coking processes as practised when applied to a comparatively limited class of coals. The percentage of workable coals available for the manufacture of metallurgical coke in the United States by previous processes has been and is small, compared to the total amount of coal.

To get a thorough understanding of the present invention a brief statement concerning the kind of coals previously considered as available for coking, and a comparison of certain characteristics thereof with those coals which have refused to yield metallurgical coke when subjected to previous processes is essential. In general coke is formed by binding the fixed carbon and ash constituents of the coal together by means of a cementing material which is made out of and from the volatile hydrocarbon contained in the original coal.

All coals when subjected to treatment in the retort and for the formation of coke, undergo certain physical and chemical changes; the result of these changes depends upon the original composition and structure of the coals and the heat treatment to which they are subjected. The general classification of coals as to whether they are "coking" or "non-coking" has been based upon results obtained when subjected to heat treatment according to previous processes. For purposes of convenience in

explanation, I shall use this terminology in this specification; but it will be understood at the beginning that the expression "non-coking" is incomplete except as coupled with a statement or explanation concerning the process to which the coal is subjected; and is, therefore, a misnomer, since coals which have refused to yield metallurgical coke under previous processes will yield metallurgical coke when treated by the present process. Accepting the previous nomenclature for simplification in explanation, I will state that research and analysis show those coals previously classed as "coking" coals fall into a very different category of structure and composition from those previously classed as "non-coking". In a general way this difference in structure and composition bears a definite relationship to geological conditions and treatment to which said coals were subjected during formation. As a rule, the coals which, by previous processes, have yielded metallurgical coke have been of the higher rank such as the semi-bituminous coals. The larger percentage of the bituminous coals have failed to yield metallurgical coke by previous processes. Such coals will yield excellent metallurgical coke in commercial quantities when subjected to treatment by this process.

To form coke of metallurgical structure the particles of carbon and other solid residuum must be bound together by a cementing material which must be formed at the right time and under the proper conditions. The two essential elements, therefore, are the solid residual matter, and a binder to join together the particles thereof into a homogeneous coke structure of proper mechanical strength and porosity. The residual matter is available from all types of coals, but a very large percentage of the coals do not have present in proper quantities nor in proper form the constituents from which to form the binding material to bind the residuum together when said coals are subjected to previous processes. But there is present in said coals the necessary constituents from and out of which the binding material is made when subjected to this process.

The binding material is not one of the constituent compounds of coal, but is evolved or formed as a product of distilla-

tion during the heat treatment and later performs its cementing functions provided the heat treatment and the process be a suitable one.

- 5 The volatile constituents contain resinous materials or resinoids and humus materials, or humoids. The cementing or binding agents are derived chiefly from the resinous materials. The process must be such as to 10 convert the resinous materials into cements or binding agents of necessary strength and quantity at the right time and in the proper manner or coke will not be formed.

If the application of heat be without reference to intensity and time, the resinoids may be vaporized and passed off slowly without much alteration in composition; consequently, but little if any cement is formed; but if rapidly heated with the 15 quantity of heat per unit of time under control they will be decomposed with consequent liberation of hydrogen gas and concentration of the carbon, so that the resinoids in their changed form will fuse or 20 become plastic or viscous and capable of acting as a cementing agent. The distilled gas carries the rapidly forming cement into the coking mass impinging it against the individual disconnected particles of residuum, surrounding them with a mass of plastic or semi-plastic or viscous material which 25 is being rapidly and continuously formed. As this action proceeds into the mass of coal, further and secondary decomposition 30 takes place with a resultant enriching and hardening effect, binding the previously disconnected residuum particles together 35 into a firm metallurgical structure or coke.

The resinous hydro-carbons melt and become plastic at 300°-to-500° C., so that they 40 are then able to flow around the particles of residuum and fill the interstices between said particles to bind them together as and when said binding material becomes sufficient in quantity and strength. At a later 45 time when the temperature of 600° to 750° C. has been reached, said resinous materials may, if present in sufficient quantities, be further decomposed with the formation of the 50 cementing agents and the consequent binding action above explained. Therefore, if the cementing function is to take place for the formation of a metallurgical structure, there must be present, when the temperature 55 of 600° to 750° C. is reached, a sufficient amount or proportion of resinous materials distributed throughout the mass and remaining in such condition that the cementing action can be performed by decomposition 60 of these bodies.

In order to bring about the ultimate formation of metallurgical coke a certain proportion of binder or cementing agent must be produced. In the so-called "coking" 65 coals, the amount of resinoids naturally

present is so large that a sufficient proportion of binding material will be formed almost without regard to the process or manner of application of heat treatment, whereas in the so-called "non-coking" coals, the 70 proportion of resinoids is so small that special consideration must be given to a process producing the heat treatment necessary to increase the production and conserve the binding material from said resinoids. 75

During the coking process, two factors or conditions diametrically opposed to the formation of coke are constantly at work tending to defeat or prevent the formation of the coke structure. The first of these is 80 the tendency of the resinoids to evaporate or vaporize and pass away from the coking mass. This is a bodily removal of material from which the binder must be formed and, therefore, directly lowers the 85 percentage of the material which should be available and which is necessary for the formation of binder.

The second factor is the tendency toward the internal destruction or alteration of the 90 resinoids in such a manner as to also lower the amount available for the ultimate production of binder. This internal destruction is a chemical reaction between the constituents of the resinoids and other elements 95 present in the coals chiefly oxygen in such form that the same can combine and re-act with the resinoids and hydrogen.

The percentage of available oxygen present in the raw material is more or less a 100 characteristic of the geological age of the material. As a rule, the coals of younger geological age run relatively higher in oxygen than those of older geological age, and it is also well understood that the coals of 105 the younger geological age cannot be coked by previously understood and practised processes.

The manner in which the percentage or amount of total oxygen varies with the geological age of the coal will be appreciated from the following comparison of oxygen content of coals of various ages:

A typical class of wood contains 83.07 parts of oxygen per 100 parts of carbon; 110

A typical class of peat contains 55.67 parts of oxygen per 100 parts of carbon;

A typical class of lignite contains 42.42 parts of oxygen per 100 parts of carbon;

A typical class of sub-bituminous coal 120 contains 21.23 parts of oxygen per 100 parts of carbon;

A typical class of bituminous coal contains 18.32 parts of oxygen per 100 parts of carbon; 125

A typical class of semi-bituminous "coking" coal contains 5.28 parts of oxygen per 100 parts of carbon; and

A typical class of anthracite contains 1.74 parts of oxygen per 100 parts of carbon. 130

This comparison clearly shows the fact that as the geological age advances the de-oxidation progresses, so that, in the higher rank coals, oxygen is only a small part of what is was in the original woody structure. This comparison also clearly shows the fact that the percentage of oxygen in the so-called coking coals is very much less than in the so-called non-coking coals.

10 The natural tendency of the available oxygen in the coal is to combine with the hydrogen and carbon of the resinous materials, breaking them down and resulting in what is, in effect, a slow combustion there-  
15 by destroying the material from which the cementing agent is formed. As the tempera-  
ture of the mass is raised in the retort, the affinity of the oxygen for the other elements becomes greater and therefore at the time  
20 when the resinous materials are ready to be converted into binding materials to per-  
form their cementing function, the available oxygen is very active chemically. There-  
25 fore, to be successful the process must be such as to quickly eliminate these oxygen compounds.

Such available oxygen as does not combine with the resinous matters is eliminated with the gaseous material. The problem, there-  
30 fore is to eliminate the oxygen with the gaseous material before it has sufficient time to decompose the bituminous or resinous mat-  
ter, so that the latter will maintain the ce-  
35 menting qualities throughout the period of carbonization. It should be further con-  
sidered that if the oxygen is in a loose combi-  
nation with the humus constituents (as is the case in the most marked degree in the humus types of coal), such as the younger and so-  
40 called "non-coking" coals, the oxygen is easily broken loose and becomes a serious factor since it can then readily combine with the hydrocarbons of the resinous materials surrounding it during the distillation period,  
45 and thus prevent their conversion into cementing materials. On the other hand, with the regular so-called "coking" coals when the oxygen is in combination with resinous constituents which have large per-  
50 centages of pitch forming hydrocarbons from which the binding materials are de-  
rived by decomposition, we have a condition in which the deleterious effect of the oxygen will not be so pronounced. This is because  
55 during the heating process the volatile hydrocarbons are evolved in percentage large enough to offset the effect of the oxygen on the cementing agents. The greater the percentage of the volatile hydro-  
60 carbon in the coal mass in proportion to the percentage of oxygen the less tendency there is to destroy that part of the residuum which becomes the binder or cementing agent by decomposition.

65 Naturally the oxygen has a strong affinity

for hydrogen present in the coal, and, therefore, the effectiveness of the oxygen in work-  
ing its destruction of the resinous matter will be interferred with to a greater or less extent by the disposable hydrogen present 70 because the combination of the oxygen with such hydrogen will result in the formation of water or moisture which will be eliminated as such with the gases and vapors with a simultaneous removal of a corresponding 75 amount of oxygen from the coking mass. Therefore, in order to examine conclusively into the effect of the oxygen on the ability to coke the coal, we must find the relation-  
ship which the oxygen and hydrogen bear 80 to each other, since that relationship is the determining element in ascertaining how much damage or destruction will be done by the oxygen present.

It must be mentioned at this point that 85 when the deleterious effect of oxygen is spoken of, and when beneficial or neutraliz-  
ing effect of the hydrogen is mentioned, reference is had to those portions of the total amount of these elements present which may 90 during carbonization combine with each other for the production of water. We must subtract, therefore, the amount of hydrogen and oxygen present in the form of water. The correctness of this reasoning will be 95 further understood when it is borne in mind that the decomposition of the resinous mat-  
ters and their conversion into cementing material takes place at a temperature of 100 600° to 750° C., so that water originally present is eliminated before the critical period is reached. Upon subtracting the amount of oxygen represented in the  $H_2O$ , we find present still a certain quantity of oxygen. This oxygen must be eliminated 105 from the coking mass or it will destroy a portion of the resinous materials which will, therefore, cease to be available when and where the cementing function is to be per-  
formed.

110 If the amount of resinous materials origi-  
nally present be relatively large as is the case in the previously classed "coking" coals, a substantial portion of it may be de-  
stroyed by this oxygen without seriously 115 interfering with the ability of the previous processes to coke the coal, because in such coals there will still be left a sufficient amount of resinous material to provide the proper amount of binder after the tempera-  
120 ture is raised to the critical point. Nature has so endowed the previously classed cok-  
ing coals with so large an amount of resinous material that a considerable portion may be destroyed by the disposable oxygen and 125 still leave enough to perform the cementing function with the production of coke even without paying special attention to the process or the manner in which the action 130 is performed.

Examination of a number of typical coals of both the so-called "coking" and "non-coking" varieties reveal the following compositions:

5

|    | Coal.              | Hydro. | Oxygen. | Dis. hydro. | Dis. ox. | Hydrogen: ox. ratio. |
|----|--------------------|--------|---------|-------------|----------|----------------------|
| 10 | Acton Basin, Ala.  | 5.15   | 8.46    | 4.94        | 6.81     | 72.5                 |
|    | Dolomite, Ala.     | 4.84   | 5.94    | 4.75        | 5.18     | 91.6                 |
|    | Wheatcroft, Ky.    | 4.53   | 8.43    | 4.25        | 6.17     | 65.2                 |
|    | Brilliant, N. Mex. | 4.97   | 8.62    | 4.81        | 7.38     | 65.2                 |
|    | Charleroi, Pa.     | 5.09   | 7.62    | 4.94        | 6.41     | 77.1                 |
|    | Connellsville, Pa. | 4.64   | 7.47    | 4.52        | 6.61     | 68.4                 |
|    | Greensburg, Pa.    | 4.82   | 5.78    | 4.71        | 4.92     | 95.7                 |
|    | Hermintie, Pa.     | 4.92   | 7.76    | 4.81        | 6.86     | 70.1                 |
|    | Millsboro, Pa.     | 4.67   | 6.43    | 4.53        | 5.30     | 85.4                 |
|    | White, Pa.         | 4.83   | 5.80    | 4.71        | 4.83     | 97.5                 |
| 15 | Fork Ridge, Tenn.  | 4.95   | 8.92    | 4.74        | 7.26     | 65.3                 |
|    | Clarksburg, W. Va. | 5.09   | 7.70    | 4.93        | 6.40     | 77.0                 |
|    | Kingmont, W. Va.   | 5.26   | 7.61    | 5.11        | 6.41     | 79.7                 |
|    | Monarch, W. Va.    | 5.04   | 8.24    | 4.88        | 6.94     | 70.3                 |
|    | Powellton, W. Va.  | 5.04   | 6.39    | 4.93        | 5.50     | 89.6                 |

20 All of the foregoing coals have in the past been considered "coking" coals and have been extensively used for the manufacture of metallurgical coke by "previous processes."

25 The following coals, on the contrary, have in the past always been classified "non-coking" and have refused to produce metallurgical coke when submitted to "previous coking processes":

30

|    | Coal.                    | Hydro. | Oxygen. | Dis. hydro. | Dis. ox. | Hydrogen: ox. ratio. |
|----|--------------------------|--------|---------|-------------|----------|----------------------|
| 35 | Benton, Ill.             | 4.90   | 11.94   | 4.47        | 8.48     | 52.7                 |
|    | Bush, Ill.               | 4.86   | 12.11   | 4.33        | 7.87     | 55.0                 |
|    | Carterville, Ill.        | 4.99   | 10.84   | 4.73        | 8.74     | 54.1                 |
|    | Centralia, Ill.          | 4.99   | 13.82   | 4.32        | 8.49     | 50.9                 |
|    | Cottontown, Ill.         | 4.69   | 12.16   | 4.23        | 8.44     | 50.1                 |
|    | Collinsville, Ill.       | 4.73   | 14.00   | 3.98        | 7.96     | 50.0                 |
|    | Donkville, Ill.          | 4.91   | 10.95   | 4.66        | 8.97     | 51.9                 |
|    | Germantown, Ill.         | 5.06   | 13.57   | 4.41        | 8.42     | 52.4                 |
|    | Harrisburg, Ill.         | 4.96   | 10.55   | 4.72        | 8.66     | 54.5                 |
|    | Herrin, Ill.             | 4.94   | 12.17   | 4.43        | 8.07     | 54.9                 |
| 40 | Lincoln, Ill.            | 4.75   | 11.15   | 4.37        | 8.12     | 53.8                 |
|    | Livingston, Ill.         | 5.11   | 14.62   | 4.32        | 8.27     | 52.2                 |
|    | Livingston, Ill. (No. 2) | 4.92   | 14.07   | 4.30        | 9.11     | 47.2                 |
|    | Marion, Ill.             | 4.92   | 12.99   | 4.26        | 7.69     | 55.4                 |
|    | Marysville, Ill.         | 4.52   | 10.23   | 4.29        | 8.40     | 51.1                 |
| 45 | New Baden, Ill.          | 4.94   | 12.20   | 4.46        | 8.32     | 53.6                 |
|    | O'Fallon, Ill.           | 5.09   | 13.86   | 4.39        | 8.28     | 53.0                 |
|    | Springfield, Ill.        | 5.00   | 12.64   | 4.43        | 8.08     | 54.8                 |
|    | Staunton, Ill.           | 5.14   | 12.32   | 4.69        | 8.74     | 53.6                 |
|    | Troy, Ill.               | 4.94   | 15.34   | 4.30        | 10.24    | 41.9                 |
| 50 | W. Frankfort, Ill.       | 4.88   | 11.25   | 4.57        | 8.77     | 52.1                 |
|    | Zeigler, Ill.            | 4.54   | 14.99   | 3.95        | 10.31    | 38.3                 |
|    | Zeigler, Ill. (No. 2)    | 5.10   | 13.53   | 4.43        | 8.19     | 54.1                 |

50 It will be found upon comparison of the above examples that in every case the total oxygen in the "coking" coals is less than 10% and is greater than 10% in each of the "non-coking" coals. This fact shows 55 the influence which the oxygen bears on the ability of previous processes to coke a given coal.

The above examples are given only as typical of the two classes of "coking" and 60 "non-coking" coals so-called, but they serve clearly to show the relationship of the hydrogen-oxygen ratio to the coking ability of previously understood and practised methods of coking. The available or dis-

substracting that portion represented by  $H_2O$ , is available to partially prevent the reaction of the oxygen on the resinous materials, because said hydrogen will combine with its equivalent weight of oxygen, and these compounds are eliminated leaving the resinous materials in the mass in such condition that if treated by the proper process they will be converted into binding material and perform their cementing function. The ratio of the disposable hydrogen to the disposable oxygen (after subtracting the water present) therefore shows definitely the existence of a necessary function of the process required for the production of metallurgical coke from that coal. This ratio is obtained by comparing the disposable hydrogen with the disposable oxygen, as shown in the examples previously mentioned herein. If this ratio exceeds 58%, the amount of hydrogen present will be sufficient to combine with and eliminate such a percentage of the oxygen that the coal is almost certain to be converted into metallurgical coke if subjected to the previously practised processes. On the other hand if this percentage be less than approximately 58%, the amount of hydrogen present will not be enough to sufficiently reduce the damaging effect of the oxygen and the coal will not be converted to metallurgical coke by previously practised methods. Therefore, in general, coals in which the hydrogen-oxygen ratio is less than 58%, must be subjected to the improved process of this invention in order to convert them into metallurgical coke.

It is to be observed that in comparing the disposable hydrogen with the disposable oxygen, for the determination of the ratios above mentioned, simply a comparison is made of the weight of disposable hydrogen as compared to the weight of disposable oxygen from the analysis of the dried coal. For example, Connellsville, Pennsylvania, coal showed 4.52 percent of hydrogen and 6.61 percent of oxygen on a dry basis, this being the available hydrogen and the available oxygen capable of reacting with each other. The ratio of 4.52 to 6.61 is 68.4%. As this is 10.4% greater than the above ratio of 58%, this coal would be classed as a "coking" coal and would yield metallurgical coke by previously practised processes. Similarly a Greensburg, Pennsylvania, coal showed 4.71 percentage of hydrogen compared to 4.92 percentage of oxygen on a dry basis, which percentages, when compared, give the ratio of 95.7%, hence this coal ranks as very high class coaking coal, according to previous classifications.

On the contrary, a Zeigler, Illinois, coal showed 3.95 percent available hydrogen, compared to 10.31 percent available oxygen on a dry basis, which percentages, when compared, show a ratio of 38.3%, hence this

coal has been classified as "non-coking." Again, a West Frankfort, Illinois, coal showed 4.57 percent available hydrogen and 8.77 percent available oxygen on a dry basis, which figures, when compared, show a ratio of 52.1%; hence this coal has also been classed as "non-coking." In fact both of these coals have been considered "non-coking" because previous processes have always failed to produce a metallurgical coke from them.

The general relationship which the total hydrogen bears to the total oxygen present in a coal, is influenced by the geological age of the coal. This is shown clearly by the following tables: Having reference to the particular samples of wood, peat, lignite, sub-bituminous coal, bituminous coal, semi-bituminous coal and anthracite previously compared on the basis of oxygen, we find—

Said wood to contain 12.18 parts of hydrogen per 100 parts of carbon;

The peat to contain 9.85 parts of hydrogen per 100 parts of carbon;

25 The lignite to contain 8.37 parts of hydrogen per 100 parts of carbon;

The sub-bituminous coal to contain 6.12 parts of hydrogen per 100 parts of carbon;

30 The bituminous coal to contain 5.91 parts of hydrogen per 100 parts of carbon;

The semi-bituminous coal to contain 4.75 parts of hydrogen per 100 parts of carbon; and

35 The anthracite to contain 2.84 parts of hydrogen per 100 parts of carbon.

From the foregoing, we find the following comparison:

|                 |                                                           |
|-----------------|-----------------------------------------------------------|
| Wood            | 12.18 of hydrogen to 83.07 of oxygen;                     |
| Peat            | 9.85 of hydrogen to 55.67 of oxygen;                      |
| Lignite         | 8.37 of hydrogen to 42.42 of oxygen;                      |
| Sub-bituminous  | 6.12 of hydrogen to 21.23 of oxygen;                      |
| Bituminous      | 5.91 of hydrogen to 18.32 of oxygen;                      |
| Semi-bituminous | "coking" coal—4.75 of hydrogen to 5.28 of oxygen; and the |
| Anthracite      | 2.84 of hydrogen to 1.74 of oxygen.                       |

Comparing the hydrogen and oxygen in each case, we find the following:

|                               |                                        |
|-------------------------------|----------------------------------------|
| Wood                          | 6.82 times as much oxygen as hydrogen; |
| Peat                          | 5.65 times as much oxygen as hydrogen; |
| Lignite                       | 5.06 times as much oxygen as hydrogen; |
| Sub-bituminous coal           | 3.46 times as much oxygen as hydrogen; |
| Bituminous coal               | 3.09 times as much oxygen as hydrogen; |
| Semi-bituminous "coking" coal | 1.11 times as much oxygen as hydrogen; |
| Anthracite                    | .61 times as much oxygen as hydrogen;  |

We may now consider another function of a process necessary for coking the so-called "non-coking" coals, viz: the prevention of 55 the loss or elimination of the hydrocarbons from which binding materials would have been formed had they been retained in the coking mass.

The resinous matters which, upon the application of a sufficient volume of heat per unit of time, may be converted into cementing material by decomposition will, if improperly heated, vaporize and pass off in a gaseous state without being decomposed sufficiently to form binding material. There-

fore, even though these materials be not destroyed by oxidation, it may still happen that they will be removed from the retort in vaporous condition and be wasted or lost without performing the cementing function. 70 This wastage can only be prevented by forcing the heat into the coal so rapidly as to decompose the resinous matter forming cementing material.

The conversion of resinous materials into 75 cementing or binding material, having reference to such portions as have not been destroyed by oxidation, consists in decomposing said resinous materials with liberation of hydrogen and deposition of carbon, or 80 the formation of cementing hydrocarbons of a higher series and with a smaller percentage of hydrogen. While there are many temperatures at which hydrogen can be separated from the hydrocarbons of coal 85 in mass carbonization, still a large part of the hydrogen is driven off at a period when the mass has reached a temperature between 600° and 750° C. indicating that this is the point of critical temperature. If the coal mass is not brought up to this temperature at a rapid enough rate, instead of eliminating the hydrogen from the carbon with the formation of binding materials and hence the formation of metallurgical coke, a large 90 part of it will volatilize thereby wasting the material from which the cement or binder would have been formed if properly decomposed. Therefore, if a coke structure is to be produced from so-called "non-coking" 100 coals, the temperature of each portion of the coal must be raised to 600° to 750° C. sufficiently fast after incipient decomposition to decompose the resinous material prior to and before it can be eliminated from the 105 coal in a gaseous state.

In the type of coals previously classed as "coking" coals, the amount or proportion of resinous materials is so large that even when the various particles are slowly heated, a sufficient amount of the resinous material will be decomposed and converted into binding material, with consequent formation of a coke structure. It will also be evident that in the case of said coals, the hydrogen-oxygen ratio is such that even though said coals be slowly heated a sufficient amount of resinous matter will remain within their body or mass undestroyed by oxidation, and capable of conversion into binding material, to enable the production of metallurgical coke regardless of the process. On the other hand in the type previously known as "non-coking" coals, the hydrogen-oxygen ratio is so small that the heat must be very rapidly 125 introduced so as to bring the coal up to decomposition temperature with consequent formation of a sufficient amount of binder before an unduly large amount of resinous material is lost by evaporation. Therefore, 130

a rapid rate of heat introduction is necessary in order to prevent destruction of the resinous materials by oxidation and to prevent wastage or elimination of said materials by 5 evaporation before decomposition.

The formation of metallurgical coke structure from the lower rank coals will also be advanced or the character of the coke improved by the additional formation of 10 binding material owing to the chemical action which I will now explain in detail.

It is the almost universal practice in retort coke ovens to transmit the heat from one or both faces of the chamber; the material 15 adjacent to or in contact with said faces is the first to be subjected to distillation. As the volatile constituents are vaporized they travel away from the heating surfaces and penetrate through the relatively cooler 20 portions of the mass undergoing treatment, and which have not yet had their temperature raised an equal amount. Some of these vapors are thus brought into contact with masses of coal below their dew point; they 25 are accordingly recondensed and deposited on the mass as tarry constituents. At a subsequent time in the process, when the heating action has still further penetrated into the mass, these same constituents are again 30 partially reëvaporated and put into vaporous condition. This results in a concentration of the hydrocarbons.

This condensing of the tarry mass results 35 in a concentration of the cementing material along a line that might be termed the outer border where the coal is being converted into coke, and, of course, said outer border is constantly traveling a greater distance away 40 from the hot wall whence the heat is derived. In the case of the high volatile, high oxygen coals, this concentration of the cementing material as it progresses away from the hot wall is very important. If the heat transmission is slow the rate of decomposition 45 is slowed down to a point where too much of these constituents will pass off in vaporous form. But if overtaken quickly by the heat of decomposition these materials will decompose forming the cement for binding 50 the fixed carbon and ash into a coke structure. This process goes on continuously from the beginning to the end of the coking cycle, there being an infinite number of periods of the evaporation of the volatile matter, its condensation at a more advanced 55 point, and its reëvaporation.

Since the heat progresses from the heating source—the wall or walls—toward that part of the mass farthest therefrom, the center of 60 the oven, it follows that the coking action throughout the mass is a progressive one, commencing at the point or points nearest the source of heat and progressing away from the same until the entire mass has been 65 penetrated by the heat, coke resulting if the

conditions be such as to bring about the proper treatment of the resinous material. The process of forming coke may be compared to a coking wave, one coming from each wall progressing through the mass, 70 traveling inwardly toward the center until its influence has been exercised throughout the mass; as the front of the wave of heat or coking action penetrates farther into the mass of coal, said mass is brought into such 75 condition that it will be converted into coke if a "regular" coking coal, but if it be a so-called "non-coking" coal the conversion into coke will not occur unless the crest of the wave reaches each point in its travel rapidly 80 enough to catch the resinous materials and convert them into cementing material by decomposition before these resinous materials could be oxidized or vaporized. The front of the wave must be steep enough to bring 85 about this conversion, or otherwise when the crest of the wave arrives the materials will have been removed from the mass.

It should here be noted that during the coking of the so-called "non-coking" coals 90 according to this process, it has repeatedly been observed that the yield of hydrogen gas and the yield of fixed carbon in the coke structure are both greater than would have been expected from a prior analysis of 95 the coal; the increased yield of hydrogen being explained by the decomposition of additional materials with consequent liberation of hydrogen; and the surplus amount of fixed carbon in the coke being explained 100 by the deposition of carbon on the residual materials simultaneously with said decomposition. This action of evaporation, condensation, and reëvaporation, results in such a concentration of tarry material just 105 in advance of the progressing wall or zone in which coking action is taking place as to actually increase the proportion of binding material to an amount greater than would naturally be expected considering the 110 original composition of the coal. Therefore, the rapid introduction of heat introduces a new step or operation, in the process of forming a coke structure, which is vital 115 to a process to be used to coke the coals previously classed as "non-coking". This is a new result following directly from the introduction of the required volume of heat per unit of time, and is in the nature of an intermediate or supplemental step.

It has been explained that at temperatures of about 600° to 700° C., the resinous materials are decomposed with consequent liberation of hydrogen and creation of new, heavier hydro-carbons having a smaller percentage of hydrogen and capable of acting as cementing materials. If the coking operations were to cease at 700° C., there would still remain considerable percentage 125 of volatile matter in the residual product, 130

so that the coke would not be fully devolatilized. Consequently, it is the practice to carry the temperature up to such point that the volatile constituents will be more 5 nearly completely eliminated, this being insured at a temperature in the neighborhood of 1100° C. The vapors or gases liberated between 700°-1100° C. serve to improve the cell structure of the coke and also 10 to harden cementing material and thus insure the formation of a hard, firm, coke structure of the physical quality to meet the needs of the blast furnace and other metallurgical uses.

15 The rate of heat application does not depend on a specific degree of temperature being used in the retort wall, but upon the rate at which the heat units necessary to perform the action are driven into the mass 20 of raw material. Of course, the temperature as an absolute amount is one of the factors bearing on the rate of introduction of heat into the mass of coal in a retort, but it is not the only factor, and, in fact, is 25 not the most important one. The rate of heat transmission from the heating gases in the combustion chamber within the walls of the retort into the mass of coal is also influenced by the resistance to the transfer of 30 heat units, so that even if very high temperatures be present in the flues or gas passages as in the old processes, it may still be impossible to secure a sufficiently rapid introduction of the required volume of heat 35 into the mass of coal, to bring about the creation of the desired product—metallurgical coke.

It has been, and still is, the universal 40 practice to use silica brick in the construction of the heating walls of the retort, and such brick has a fusion temperature of approximately 1750° C. so that this is the absolute upper limit of temperature, and, in fact, it is not practicable to use temperature 45 above 1560° C. in the flues or gas passages, since a sufficient margin of safety must be provided. Experience has shown that even when using temperatures as high as 1650° C. in previous processes it has been 50 impossible to secure a sufficiently rapid introduction of heat units into the coking mass to bring about the creation of the coking structure, in the so-called "non-coking" coals.

55 We must, therefore, look to the other factor in order to solve the problem of introducing the heat in a sufficiently rapid manner to bring about the desired result. This other factor is the heat absorbing and 60 transmitting capacity of the walls for the transfer of heat units from the heating gases to the interior of the coal mass. By increasing the heat absorbing and transmitting powers of these parts to a sufficient degree, it will become possible to secure a suf-

ficiently rapid transfer of heat units into the coal mass without the use of high temperatures. In this connection it should be remembered that it is not necessary to attain high temperatures in the coking mass 70 itself, since the entire coking process can be completed in any given particle of coal at a temperature of 1000° C. or less. In fact, it would be desirable to be able to perform the entire process with temperatures in the combustion chamber of not to exceed, for example, 1000° C. which is being done by this process, since the wear and tear and the deterioration would be correspondingly minimized. 80

The rate of heat transmission into the coking mass has, of course, reference to each and every particle which is to be made to yield to the coking function. The retort has a certain width, and it is customary 85 to introduce the heat into the retort by heating one or both of the walls. When both of the walls are heated, the heat travels inwardly from each of them toward the center of the retort, and therefore the coking 90 process, commencing at the walls, travels inwardly toward a dividing surface approximately at the middle of the retort, and which is more or less in the form of a plane. Since it is practically the universal custom 95 to heat both sides of the retort, the heat traveling toward the middle of the oven from each side, I will hereafter make reference to such construction and describe such operation, but in so doing I wish it distinctly understood that this is done simply 100 as a matter of convenience in this specification, and not as a matter of limitation, since the same principles would apply if the retort were to be heated on only one side or 105 face, in which case the coal adjacent to the other side or face would be the last to reach the conclusion of the process.

As the heat travels from the walls toward the center of the oven, it must pass through 110 a constantly increasing thickness of material, be the said material coal, coke, or coal at some intermediate stage of transformation. All of these materials are relatively poor conductors of heat and, therefore, the rate of heat transfer to the middle 115 of the oven is greatly impeded by the intervening material.

Assuming the temperature in the heating walls to be not greater than a predetermined 120 amount, the width of the oven would, therefore, be limited to such a distance as would permit of a sufficiently rapid raising of the temperature of the middle portion of the coking mass. This means that the tendency 125 in the design and construction of the ovens should be toward the narrower retort in order to satisfactorily handle the "non-coking" coals. Reduction in the width of the retort entails corresponding reduction 130

in cubical capacity and corresponding reduction in the amount of charge which can be coked at one operation. As a matter of economy in operation and earning capacity of the plant, the charge should be kept as large as possible. The volume of the retort can be only increased by increasing its height and length, assuming that its width has been fixed. The height and length of the retort are limited, among other things, by the ability to uniformly heat the entire surface by the heating gases. In those cases in which the gases travel downwardly through the heating walls, the height is so limited. The length of the oven is largely limited by the ability to push the completed coke out of the retort at the termination of the operation, since the total friction or resistance to pushing is increased by increase of length, and since there is a very large side thrust exerted on the walls of the retort tending to displace them or separate them farther apart.

The use of a relatively narrow retort is also consistent with the previously explained evaporation, condensation and re-evaporation of the volatile constituents which constitute a portion of the cementing materials. This previously explained action of evaporation, condensation and re-evaporation tends to concentrate the cementing agencies in that portion of the coal mass at the center of the chamber, and thereby correspondingly improve the conditions existing in that portion of the chamber, so that it becomes possible to carry the coking action through the entire mass of the material, notwithstanding the fact that the rate of heat transfer in the middle portion of the chamber is necessarily slower than in those portions adjacent to the walls, the difference in rate of heat transfer being compensated for by the condensation and re-evaporation of the cementing materials.

This ability to carry the coking operation throughout the entire width of the chamber is also aided by another factor, which is the fact that some chemical re-actions of the coal in process of carbonization are exothermic while others are endothermic. The re-actions of formation of such bodies as carbon dioxide, carbon monoxide, methane, water and ammonia are exothermic in nature, resulting in giving off considerable quantities of heat, while the actions of generating such bodies as benzene, ethylene, carbon bisulfid, cyanogen and tar vapors are endothermic in nature, necessitating the absorption of large amounts of heat in order to bring them about. The heat from the exothermic re-actions is less than that necessary for the endothermic re-actions, and the difference must, of necessity, be supplied by the heat coming from the walls of the retort. Investigation has shown that at

temperatures between 600° to 750° C. practically all types of coals display exothermicity. Since the critical temperature for the fixing of the cementing agency is in the neighborhood of 600° to 750° C., it follows that at the very time when the resinous materials are being converted into cementing material exothermic re-actions occur, with a corresponding improvement of the conditions under which the conversion may take place. By rapidly raising the temperature to this critical point, not only is it possible to bring about the conversion of the cementing material, but also advantage may be taken of the exothermicity to assist the re-action.

The heat for the coking process comes, in the first instance, from the heating gases traveling through the flues or passages. Thence it is transferred to the oven structure and through the same to the surface of the retort. If there be no charge of coal in the chamber, the walls and oven structure will in time attain the temperature closely approximating that of the heating gases flowing through them, and will have stored within them a certain amount of heat as a reservoir or reserve which may be drawn upon when the powdered or fine coal is charged into the oven. As soon as the coal is charged, there will commence a rapid transfer of heat from the walls and oven structure into the coal, with a consequent demand upon said reserve or supply. This demand will result in a corresponding lowering of the temperature of the walls and structure, and (disregarding for the moment the extraction of fresh heat from the heating gases), the ability to raise the temperature of the raw material will depend chiefly upon the amount of this reserve as compared to the amount of coal in the retort. If the coal be of the so-called "non-coking" variety, its temperature must be rapidly raised to the point at which the binding materials are formed, and this means that a large reserve supply of heat should be available in the oven structure. The amount of this reserve of heat is partially measured by a comparison of the weight of the walls and hot structure with the weight of the coal, taking account of the specific heat of the walls and structure. In the case of silica brick constructions, this specific heat averages approximately .20 as compared to water as 1.00. In actual practice, the heating gases are at all times transferring live heat to the walls of the structure so that the reserve is supplemented.

As long as there remains a zone of coal which is not fully coked, the temperature of the coking mass cannot rise greatly above the point at which decomposition takes place, although it will be understood that necessarily the mass close to the walls is always hotter than the "core" or central por-

tion of the mass. As soon as the coking process has been completed by practically complete elimination of the volatile constituents, the temperature of the entire mass 5 will rise rapidly, thus showing that the operation has been completed and that the coke should be "pushed".

The curves in the accompanying figure are typical of the temperature changes taking place in a typical retort oven when 10 using the present process for coking the so-called "non-coking" coals. These curves are 15 illustrative of action at various points in the retort, and are in no sense to be considered as limitations upon the use or practice of 20 the present invention and process, or as being in any sense a narrowing of the scope of the present invention which is defined in and covered by the claims.

25 Bearing this in mind, curve 10 shows a typical variation of wall temperature with respect to time, and curves 11, 12, and 13, respectively, show typical temperature variations with respect to time at a point two 30 inches from the hot wall, farther in from the wall surface, and at the center of the mass.

The following conditions are assumed in connection with these curves, such assumption 35 also being simply for purposes of illustration: initial wall temperature 1200° C. just after introduction of the charge; initial coal temperature 20° C. The first action taking place at any point within the mass 40 is the elimination of the original moisture.

It is observed that all of the curves rise 45 rapidly to the knee designated at the point A where each curve becomes practically flat until the original moisture has been evaporated. Thereafter, the individual curves 50 rise more or less rapidly. The curve 11 rises most rapidly because it represents a point closest to the wall. It reaches a knee at the point B representing approximately 700° C., 55 where it rests for a considerable interval of time, as shown by the relatively flattened portion C. During this interval the resinous 60 matters are being decomposed with consequent liberation of hydrogen and formation of binding or cementing materials.

During this time, also, additional heat is 65 being transmitted to points farther from the wall and nearer the core. The curve 12 rises somewhat slower and at a later time to a knee at the point D representing approximately 700° C., where it also rests for an 70 interval of time during the period of decomposition and formation of binding material.

The curve 13 representing the conditions 75 at the core rises latest to the point E being somewhat lower in temperature than the knees B and D, since (on account of the evaporation of tarry matters from the zones 80 nearer the wall and their condensation near

the core), the conditions at that point are more favorable for the production of binding or cementing agents. On account of such concentration of tarry material and consequent improvement of the coking conditions, it is unnecessary to raise the temperature of the core as rapidly or to the same degree in order to secure a sufficient amount of binding material for the formation of the metallurgical coke structure. 75

After the decomposition action, the temperature begins to rise substantially at the point F, commencing first in the material closest to the wall and progressing toward the central zones. This rise of temperature 80 at each zone continues to the point G represented by 1000°-1100° C., and between the points F and G higher boiling hydro-carbons are being liberated and broken up or 85 delivered from the mass so as to complete the devolatilization of the coke structure. Therefore, the oven should be pushed substantially at the time represented by the point G. After this point is reached, the temperature rises rapidly without corresponding 90 beneficial result, and there is apt to be an overheating of the oven walls, since there is no volatile matter present to absorb the heat and hold down the temperature.

Substantially between the points B and 95 F, there takes place the decomposition of resinous materials with conversion of binding or cementing material. The endothermic actions predominate in this portion 100 of the process. Subsequently the exothermic actions occur.

The important relationship which the heat reservoir in the wall bears to the process of this invention for the production of metallurgical coke from the so-called "non-coking" coals, is well illustrated by the curve 10, and its relationship to the other curves of this figure. It is observed from the introduction of the coal down to the point represented by J, curve 10 is falling, indicating 105 that the wall is giving up heat previously stored in it, and is, therefore, enabling a more rapid penetration of the heat into the coking mass. The point J is opposite to that portion of the curves 11, 12 and 13 110 which represent decomposition of resinoids and the formation of binding material. The rapidity with which the curves 11, 12 and 13 are brought up to this decomposition temperature is largely dependent upon the delivery of heat previously stored in the walls. This, in turn, depends largely on the mass 115 of the walls and arrangement of the heating structure as compared to the mass of coal in the charge. 120

It is observed that the curve 10 rises after reaching the point J showing that after practically the entire mass has been raised to the decomposition temperature, where it rests more or less uniform for a period of 130

time, the heating gases in the walls are giving up their heat to the walls more rapidly than the heat is being withdrawn from the walls by the coking mass. Consequently 5 when the end of the operation is reached, the walls are restored practically to their maximum temperature preparatory to the next charge.

If there be provided approximately 3.8 10 pounds of wall and wall structure (arranged to give up its heat rapidly on demand) per pound of coal in the retort, there will be a sufficient reserve of heat available to coke the high volatile high oxygen "non-coking" 15 coals by the practice of the present invention, provided the nature of the wall structure be such as to rapidly absorb heat from the heating gases, and also provided that the weight of coal in the retort be not excessive 20 as compared to the area of the walls of the retort. Of course, if other material than silica be used for the walls and hot structure, account should be taken of its specific heat and conductivity as compared to that of 25 silica and the weight factor correspondingly modified in inverse ratio which the average specific heat of such other material bears to that of silica which averages .20.

In order to most perfectly transfer the 30 heat from the gases into the wall structure, the passages in said structure should be relatively complex and small enough to insure a perfect contact of all portions of the gas with the wall structure during their travel. 35 The smallness of these passages is to some extent limited by the ability to provide sufficient cross sectional area for the transfer of the necessary volume of gases without unduly limiting or impeding its flow. However, 40 if the total cross sectional area of the passages be made approximately equal to that of the intervening blocks or structure, a very satisfactory proportion will be realized for the process of the present invention.

45 The ability of the coal mass to absorb the heat from the walls and thus bring about the rapid rise of temperature and rapid decomposition combined with the concentration and evaporation of tarry materials is 50 largely dependent upon the mass of coking material per unit area of heating surface in the retort. This amount or ratio should be kept as small as possible in order to reduce as much as possible the demand for heat 55 from each unit of area of heating surface. This reduction, however, means a corresponding narrowing of the retort. If the width of the retort be made from 12 to 16 inches, it will be found possible to coke practically 60 all of the bituminous "non-coking" coals by the process of the present invention. It may also be stated that if the amount of coal in the retort be made approximately 29-30 pounds per square foot of heating

surface of a retort, such coals may be coked 65 by the process of the present invention.

The introduction of heat into the coking mass from the live heating gases depends somewhat upon the ratio of mass of coal in the retort as compared to the area of said 70 gas passages. It is desirable to keep this ratio as small as possible so as to enable the most rapid introduction of heat into the coal from the heating gases. If the structure be such that approximately 12 to 13 pounds of 75 coal be present in the retort per square foot of surface in the heating gas passages, practically all of the bituminous coals can be coked by the process of the present invention. In like manner it is desirable that the 80 area in the heating gas passages should be as large as possible compared to the area of heating surface in the retort. If the area exposed to the heating gases in the passages be approximately 2.25-2.50 times as large 85 as the area of heating surface in the retort, it will be possible to coke practically all of the bituminous coals by the process of the present invention.

Where, in the claims, I use the expression 90 "in raw condition and substantially without admixture of foreign substance," I mean that the coal is inserted or introduced into the retort in substantially its raw form or condition and without the admixture of foreign substance for the purpose of providing material from which to secure or form the binder or cementing agent. By the expression "raw condition" or like expressions, I do not mean that the coal is not broken up 100 or even pulverized, since the raw coal may, of course, be broken up or pulverized without modifying its chemical condition and properties, but rather I mean that the coal is introduced into the retort without previous coking treatment or the like. Naturally 105 the exact degree of fineness or comminution of the coal will depend somewhat upon the wishes of the operator, but the essential thing under the claims mentioned is that the 110 coal should be used substantially without any foreign substance, and without prior coking or other treatment. In its broader aspect, however, as set forth in other claims, my invention and process are applicable to 115 coking material formed either of a mixture of a non-coking coal having a low content of hydrogen relative to its content of oxygen with a coal of higher hydrogen content, or a mixture of a non-coking coal of low hydrogen content with foreign substances of 120 higher hydrogen content, such as various bituminous or asphaltic substances. In particular, and by way of illustration, my invention and process may be successfully used 125 to produce metallurgical coke from a mixture of lignite coal, having a low hydrogen content, with a coal of higher hydrogen con-

tent even though the proportions and character of the two be such that the hydrogen content of the resulting mixture falls considerably below the minimum hydrogen content of coals heretofore considered cokable coals.

I wish it distinctly understood that the mention of ratios and weights and areas as above given is purely illustrative and is not to be in any sense considered as a limitation on the process of the present invention.

I wish also to emphasize the presence or existence of a new result in the process of coking the high volatile high oxygen bituminous coals by the rapid introduction of heat. This results in the larger concentration of the tarry resinous matters (from which the binder or cementing material is derived) along a progressive zone within the retort. The temperature of this zone is raised so rapidly to the necessary degree for decomposition of said tarry matters that the destruction by oxidation or elimination by evaporation does not prevent the formation of the metallurgical coke structure.

I am aware that it has been proposed, as in the Engelmann patents (Nos. 136,592 and Reissue No. 5,486) to coke lignitic coal by mixing therewith a sufficient quantity of coking coal, or of bituminous or asphaltic substances, to produce a mixture approximating the character of bituminous coking coals; but by my novel process I am enabled to produce metallurgical coke not only from coals heretofore considered non-cokable, as described in the foregoing specification, but I am enabled to produce metallurgical coke from coking mixtures, such as a mixture of lignitic coal with other coal of a higher hydrogen content, which do not approximate the character of bituminous coking coals, but which, on the contrary, like the sub-bituminous, bituminous and semi-bituminous coals referred to in the foregoing specification, fall considerably below the content of hydrogen relatively to oxygen that is found in coals heretofore considered cokable.

I claim:

1. The process of treating coals to produce metallurgical coke in which said coals the amount of disposable hydrogen does not exceed approximately fifty-eight percent. of the amount of disposable oxygen, which consists in charging such coal into a closed retort and introducing heat into the coal mass through the medium of the retort and with the exclusion of air, the heat being introduced from the retort so rapidly that the temperature of each portion of the mass is raised to approximately seven hundred degrees centigrade before oxidation of the resinous constituents by the oxygen in the coal, whereby said resinous constituents are

decomposed with the formation of cementing material and liberation of hydrogen in each portion of the mass before the destruction of the resinous constituents in such portion by oxidation, and with consequent production of a metallurgical coke structure. 65

2. The process of treating coals to produce metallurgical coke in which said coals the amount of disposable hydrogen does not exceed approximately fifty-eight percent. of the amount of disposable oxygen, which consists in charging the same into a closed retort and introducing heat into the coal mass through the medium of the retort and with the exclusion of air, the heat being introduced so rapidly that the temperature of each portion of the mass is raised to the temperature of decomposition of its resinous constituents before oxidation of such resinous constituents by the oxygen in the coal, whereby said resinous constituents are decomposed with the formation of cementing material and liberation of hydrogen in each portion of the mass, before the destruction of the resinous constituents in such portion by oxidation and with consequent production of a metallurgical coke structure. 70

3. The process of treating coals to produce metallurgical coke in which said coals the amount of disposable hydrogen does not exceed approximately fifty-eight percent. of the amount of disposable oxygen, which consists in charging the same into a closed retort and introducing heat into the coal mass through the medium of the retort and with the exclusion of air, the heat being introduced so rapidly that the temperature of each portion of the mass is raised to the point of decomposition of its resinous constituents before oxidation of said constituents by the oxygen in the coal, whereby the particles of coal are cemented together into a metallurgical coke structure before destruction of said resinous constituents by oxidation. 95

4. The process of treating high volatile, high oxygen, bituminous coals for the production of metallurgical coke, which consists in charging the same in raw condition and substantially without admixture of foreign substance into a closed retort and introducing heat into the coal mass through the medium of the retort and with the exclusion of air, the heat being introduced so rapidly that the temperature of each portion of the mass is raised to the point of decomposition of its resinous constituents before oxidation of said constituents by the oxygen present in the coal, whereby said resinous constituents are decomposed with the formation of cementing agents and liberation of hydrogen in the mass before the destruction of the resinous constituents in such portion by oxidation and with conse- 110  
115  
120  
125

quent production of a metallurgical coke structure.

5. The process for the treatment of high volatile, high oxygen, bituminous coals having a relatively small percentage of resinous constituents present in their mass, which consists in charging the mass in raw condition and substantially without admixture of foreign substance into a closed retort and 10 introducing heat into the coal mass through the medium of the retort and with the exclusion of air, the heat being introduced so rapidly that the temperature of each portion of the mass is raised to the point of 15 decomposition of its resinous constituents before excessive oxidation of said resinous constituents by the oxygen present in the coal, whereby sufficient amounts of said resinous constituents are decomposed in all 20 portions of the mass of coal with consequent production of cementing agents to bind the particles of material into a metallurgical coke structure.

6. The process of treating coals to produce metallurgical coke in which said coals the amount of disposable hydrogen does not exceed approximately fifty-eight percent of the amount of disposable oxygen, which consists in charging the same into a closed 25 retort and introducing heat into the coal mass through the medium of the retort and with the exclusion of air, the heat being introduced so rapidly that the temperature of each portion of the mass is raised to the 30 point of decomposition of its resinous constituents before excessive oxidation of said resinous constituents by the oxygen present in the coal, whereby sufficient amounts of said resinous constituents are decomposed in 35 all portions of the mass of coal with consequent production of cementing agents to bind the particles of material together into a 40 metallurgical coke structure.

7. The process of treating bituminous 45 coals in which said coals the amount of disposable hydrogen present does not exceed approximately fifty-eight percent of the amount of disposable oxygen present for the production of metallurgical coke from 50 such coals, which consists in charging the same into a relatively narrow retort and delivering heat into the coal from the retort with the exclusion of air, the heat being supplied from the sides of the retort and 55 proceeding toward the middle of the retort from opposite directions to thereby volatilize the low boiling hydrocarbons commencing at the sides and advancing toward the center, those hydrocarbons which are first 60 volatilized being recondensed on the interior cooler portions of the mass with concentration of said hydrocarbons in such portions, and being subsequently evaporated as the heat penetrates into the mass, the heat 65 penetrating into the mass so rapidly as to

raise the temperature of each portion of the mass to the point of decomposition of the resinous constituents in such portion before their excessive destruction by oxidation taking account of their amounts present by previous recondensation, with consequent formation of cementing material from such hydrocarbons, whereby there is created a progressive wave of cementing action within the mass commencing at the walls and traveling so rapidly toward the center of the retort as to form cementing agents at each point by decomposition prior to excessive destruction of said hydrocarbons by oxidation.

8. The process of treating high volatile, high oxygen, bituminous coals for the production of metallurgical coke, which consists in charging the same in pulverized condition raw and substantially without admixture of foreign substance into a relatively narrow retort and delivering heat into the coal from the retort with the exclusion of air, the heat being supplied from the sides of the retort and proceeding toward the middle of the retort from opposite directions, to thereby volatilize the low boiling hydrocarbons commencing at the sides and advancing toward the center, those hydrocarbons which are first volatilized being 90 recondensed on the interior cooler portions of the mass with concentration of said hydrocarbons in such portions, and being subsequently evaporated as the heat penetrates into the mass, the heat penetrating into the 95 mass so rapidly as to raise the temperature of each portion of the mass to the point of decomposition of the resinous constituents in such portion before their excessive destruction by oxidation, taking account of 100 their amounts present by previous recondensation, with consequent formation of cementing agents from such hydrocarbons, whereby there is created a progressive wave 105 of cementing action within the mass commencing at the walls and traveling so rapidly toward the center of the retort as to form cementing material at each point by decomposition prior to excessive destruction of said hydrocarbons by oxidation.

9. The process of treating coals to produce metallurgical coke, in which said coals the amount of disposable natural hydrogen does not exceed approximately fifty-eight per cent. of the amount of disposable natural oxygen, which consists in charging the same into a retort and introducing heat into the coal mass through the medium of the retort, the heat being introduced so rapidly that the temperature of the mass is raised to 125 the temperature of decomposition of its resinous constituents before oxidation of the entire content of such resinous constituents, whereby a sufficient residue of such resinous constituents is decomposed to form the nec- 130

essary quantity of cementing material to afford a binder for the consequent production of a metallurgical coke structure.

10. The process of treating high volatile, high oxygen, bituminous coals for the production of metallurgical coke, which consists in charging the same in raw condition and substantially without admixture of foreign substance into a retort and introducing 10 heat into the coal mass through the medium of the retort, the heat being introduced so rapidly that the temperature of the mass is raised to the temperature of decomposition of its resinous constituents before the oxidation 15 of the entire content of such resinous constituents, whereby a sufficient residue of such resinous constituents is decomposed to form the necessary quantity of cementing agents to afford a binder for the consequent 20 production of a metallurgical coke structure.

11. The process of treating coals to produce metallurgical coke in which said coals the amount of disposable hydrogen does not exceed approximately fifty-eight percent. 25 of the amount of disposable oxygen, which consists in charging the same into a retort and introducing heat into the coal mass through the medium of the retort, the heat being introduced so rapidly that the temperature of the mass is raised to the temperature of decomposition of its resinous constituents before excessive evaporation thereof, whereby a sufficient residue of said resinous constituents is decomposed in contact 30 with the humous bodies in each portion of the mass to bind said humous bodies together with the consequent production of a metallurgical coke.

12. The process of treating high volatile, high oxygen, bituminous coals for the production of metallurgical coke, which consists in charging the same in raw condition and substantially without admixture of foreign substance into a retort and introducing 45 heat into the coal mass through the medium of the retort, the heat being introduced so rapidly that the temperature of the mass is raised to the temperature of decomposition of its resinous constituents before excessive 50 evaporation thereof, whereby a sufficient residue of said resinous constituents is decomposed in contact with the humous bodies in each portion of the mass to bind said humous bodies together with the consequent 55 production of a metallurgical coke.

13. The process of treating high volatile, high oxygen, bituminous coals for the production of a maximum yield of coke, which consists in charging the coals into a retort 60 in raw condition and substantially without admixture of foreign substance and introducing heat into the coal mass through the medium of the retort so rapidly that the temperature of the mass is raised to the 65 point of decomposition of the resinous con-

stituents prior to their excessive dissipation by evaporation, whereby a maximum portion of said resinous constituents is decomposed with consequent deposition of carbon and increased yield of coke.

14. The process of treating high volatile, high oxygen, bituminous coals for the production of metallurgical coke, which consists in charging the same into a retort of sufficient mass as compared to the mass of 70 coal charged into it and of suitable temperature to insure the introduction of heat into the coal from the retort with sufficient rapidity to raise the temperature of the coal to the point of decomposition of its resinous 75 constituents before oxidation of the entire content of such resinous constituents, whereby a sufficient residue of said resinous constituents is decomposed to form the necessary quantity of cementing material to afford 80 a binder with the consequent production of a metallurgical coke structure.

15. The process of treating high volatile, high oxygen, bituminous coals for the production of metallurgical coke, which consists in charging the same into a retort of sufficient mass as compared to the mass of coal charged into it and of suitable temperature to insure the introduction of heat into the coal from the retort with sufficient 90 rapidity to raise the temperature of the coal to the point of decomposition of its resinous constituents before oxidation of the entire content of such resinous constituents, whereby a sufficient residue of said resinous constituents is decomposed in the presence of 95 the humous constituents to form the necessary quantity of cementing agents to afford a binder with the consequent production of a metallurgical coke structure.

16. The process of treating high volatile, high oxygen, bituminous coals for the production of metallurgical coke, which consists in charging the same into a retort of sufficient mass as compared to the mass of 100 coal charged into it and of suitable temperature to insure the introduction of heat into the coal from the retort with sufficient rapidity to raise the temperature of the coal to the point of decomposition of its resinous constituents before excessive dissipation by 105 evaporation of said resinous constituents, whereby a sufficient quantity of said resinous constituents is decomposed in the presence of humous constituents to afford a binder with the consequent production of a metallurgical coke structure.

17. The process of treating high volatile, high oxygen, bituminous coals for the production of metallurgical coke, which consists in charging the same in raw condition and substantially without admixture of foreign substance into a retort and introducing 110 heat into the coal mass through the medium of the sides of the retort, the heat 115

120

penetrating the mass with sufficient rapidity to raise the temperature at each point within the mass to the temperature of decomposition of its resinous constituents prior to excessive oxidation and excessive dissipation by evaporation of the resinous constituents at that point, to thereby form a sufficient amount of cementing material at each point to bind the entire mass together into a metallurgical coke structure.

18. The process of treating high volatile, high oxygen, bituminous coals for the production of metallurgical coke, which consists in charging the same into a retort of suitable temperature and thereafter introducing heat into the charge through the medium of the retort, the mass of the retort including its heating walls being approximately 3.8 times as great as the mass of the material charged into the retort, taking account of the specific heat of the retort materials, whereby there is insured the introduction of heat into the coal from the retort with sufficient rapidity to raise the temperature of the coal to the point of decomposition of its resinous constituents before excessive dissipation by evaporation of said resinous constituents, whereby a sufficient quantity of said resinous constituents is decomposed in the presence of humous constituents to afford a binder with the consequent production of a metallurgical coke structure.

19. The process of treating high volatile, high oxygen, bituminous coals for the production of metallurgical coke, which consists in charging the same into a retort of suitable temperature and thereafter introducing heat into the charge through the medium of the retort, the mass of the retort including its heating walls being approximately 3.8 times as great as the mass of the material charged into the retort, taking ac-

count of the specific heat of the retort materials, and the mass of coal in the retort being approximately 29-30 pounds per square foot of heating surface of the retort.

20. The process of treating high volatile, high oxygen, bituminous coals for the production of metallurgical coke, which consists in charging the same into a retort of suitable temperature and thereafter introducing heat into the charge through the medium of the retort, the mass of coal in the retort being approximately 29-30 pounds per square foot of heating surface of the retort.

21. The process of treating high volatile, high oxygen, bituminous coals for the production of metallurgical coke, which consists in charging the same into a retort of suitable temperature and thereafter introducing heat into the charge through the medium of the retort, the retort being provided in its side walls with passages for heating gases, the mass of coal in the retort being approximately 12-13 pounds per square foot of heated surfaces of said passages.

22. The process of treating high volatile, high oxygen, bituminous coals for the production of metallurgical coke, which consists in charging the same into a retort of suitable temperature and thereafter introducing heat into the charge through the medium of the retort, the mass of coal in the retort being approximately 29-30 pounds per square foot of heating surface of the retort, the retort being provided in its side walls with passages for heating gases, and the mass of coal in the retort being approximately 12-13 pounds per square foot of heated surfaces of said passages.

ARTHUR ROBERTS.

Witness:

THOS. A. BANNING, Jr.